

L. KIRSCHBRAUN.  
ASPHALTIC PRODUCTS AND PROCESS OF MAKING THE SAME.  
APPLICATION FILED MAR. 29, 1912.

1,194,750.

Patented Aug. 15, 1916.



# UNITED STATES PATENT OFFICE.

LESTER KIRSCHBRAUN, OF CHICAGO, ILLINOIS.

## ASPHALTIC PRODUCTS AND PROCESS OF MAKING THE SAME.

1,194,750.

Specification of Letters Patent. Patented Aug. 15, 1916.

Application filed March 29, 1912. Serial No. 687,021.

To all whom it may concern:

Be it known that I, LESTER KIRSCHBRAUN, a citizen of the United States, residing in the city of Chicago, county of Cook, and 5 State of Illinois, have invented certain new and useful Improvements in Asphaltic Products and Processes of Making the Same, of which the following is a specification.

This invention relates to improvements in 10 asphaltic products and processes of making the same and refers more particularly to making new and improved asphaltic products from semi-asphaltic base petroleum residuum, *i. e.*, the heavy residues left after 15 removing the naphthas, burning oils and portions of the lubricating oils, until the residuum referred to has a gravity of about 12 to about 24 degrees Baumé.

Among the salient objects of the invention 20 are to so treat petroleum residuum of the character referred to as to remove from such residuum the greater part of the vaseline, paraffin and analogous hydrocarbons contained therein and without any material de- 25 composition; to provide a process which will convert the residuum of the character in question into a new asphaltic product which will have a remarkable degree of ductility and cementitiousness as well as other char- 30 acteristics not found in asphaltic products heretofore made from petroleum residuum of the character in question; to provide a process for producing products of the above mentioned character in which semi-asphaltic 35 base petroleum residuum is subjected to the combined action of heat and superheated steam in a still at temperatures below the boiling temperature of the residuum whereby the aforesaid hydrocarbons are removed 40 at comparatively low temperatures, *i. e.*, below the temperatures of ordinary fractional distillation; to provide a process in which the vapor pressure of the paraffin or vaseline hydrocarbons is in effect, so raised that these 45 hydrocarbons will be removed from the residuum at temperatures sufficiently low to obviate any danger of decomposition or otherwise injuring the asphaltic hydrocarbons, the residuum by such treatment being so 50 modified as to produce a new asphaltic product; to provide a process in which the paraffin, vaseline and other analogous hydrocarbons are removed from the residuum without being decomposed or cracked, thus 55 avoiding the addition of deleterious sub-

stances in the resultant product; to provide a process which is simple and economically operated and necessitates only the use of heat and superheated steam; and in general to provide a new and improved product of 60 the character referred to.

The invention consists in the matters hereinafter described and more particularly pointed out in the appended claims.

In present commercial practice crude petroleum is fractionally distilled by the use of saturated steam and heat. I am aware that various writers on the distillation of crude petroleum have discussed the use of air, superheated steam and inert gases. I 65 am also aware that artificial asphalts and asphaltic fluxes have been made from petroleum residuum or tar by subjecting heated residuum to the action of air, sulfur or saturated steam. In some cases, as for 70 example, when air is used, the residuum has been heated to such a degree as to cause material distillation, the air causing certain chemical re-actions resulting in cracking and the production of a solid residue. In 75 other cases where air has been used the temperature has been kept sufficiently low to avoid cracking or material distillation and the mass has been solidified by oxidation of the residuum, the latter being blasted with 80 copious amounts of air. The present invention however has nothing to do with the treatment of crude petroleum nor does it have anything to do with the production of 85 asphaltic products or asphaltic fluxes of the character last referred to. Products produced by the use of air or sulfur are not in any sense analogous or equivalent to products produced by my process. The former contain the greater proportion of the par- 90 affin and vaseline and analogous hydrocarbons contained in the original residuum or else contain their cracked or decomposed residues. By my process such hydrocarbons are removed without cracking or decomposi- 95 tion. These prior art products are relatively non-ductile, have excessively high melting points with reference to their consistency, are more or less greasy and cheesy in character, and if subjected to too high a 100 degree of heat when being made are crumbly, brittle and non-homogeneous. The air blown asphalts for example, exhibit as one of their main characteristics a great inert- 105 ness as to changes in their consistency under 110

extremes of temperature, and are extremely viscous in character when melted. The present process produces a product which has characteristics opposite from those mentioned in the foregoing sentence; my products having an unusual degree of ductility, in many cases having an elongation of more than one hundred times their cross section at normal temperature, *i. e.*, 77° F. and having a high degree of adhesiveness and cementitiousness not found in asphaltic products heretofore made from semi-asphaltic base petroleum residuum.

As stated, the present invention is directed primarily to a process of treating semi-asphaltic base residuum so as to remove the greater part of the vaseline, paraffin and analogous hydrocarbons contained in the residuum and in such a way as to provide a new asphaltic product. Semi-asphaltic base residuums are obtained from the mid-continent and Gulf fields and more particularly from the Illinois, Kansas, Texas, Louisiana, Oklahoma and Wyoming and also the Mexican fields, although there may be other fields from which semi-asphaltic base oils may be obtained. By semi-asphaltic base residuum is meant such petroleum residuum as contains a substantial percentage of asphaltic hydrocarbons in addition to paraffin and analogous saturated hydrocarbons which are present in petroleum. While asphaltic products have heretofore been made from both asphaltic and semi-asphaltic base residuums by the use of heat and air or heat and other oxidizing agent such processes and products are not in any sense analogous to mine as they cause certain chemical reactions not found in my process and produce products radically different from the products produced by the present invention. It is also true that asphaltic products have heretofore been made from a strictly asphaltic base residuum by the use of heat and saturated steam, my new product however, can not be made from semi-asphaltic base residuum by the use of saturated steam for the reason that in order to distil off the paraffin and vaseline hydrocarbons with saturated steam it is necessary to raise the temperature so high that cracking or decomposition results. Nor can these hydrocarbons be distilled by straight distillation with heat alone without decomposition as the paraffin and vaseline hydrocarbons will decompose at temperatures below that at which they can be removed from the still.

I have discovered that by subjecting semi-asphaltic base residuum of the character in question to the action of large quantities of superheated steam at a relatively low pressure the major portion of the paraffin and vaseline (amorphous paraffin) hydrocarbons contained in the residuum can be removed

from the still without decomposition, the temperature being however, considerably below that at which the hydrocarbons would decompose. The paraffin and vaseline hydrocarbons referred to are those saturated hydrocarbons which are non-removable by concentrated sulfur acid, (H<sub>2</sub>SO<sub>4</sub>); it being understood that the unsaturated hydrocarbons are removable by concentrated sulfuric acid. By such process my new product of the character heretofore referred to is obtained. The process will perhaps be more readily understood by referring to the accompanying drawing in which—

Figure 1 is a longitudinal sectional view of an apparatus suitable for carrying out the present invention; Fig. 2 is a detailed view of one of the branch steam pipes with which the still is equipped.

Referring now to the drawings—1 designates a supply pipe leading from any suitable source of steam supply, such as exhaust steam or low pressure steam from a boiler. This pipe 1 is connected to steam coil 2 of a suitable superheater 3, whereby the exhaust steam or low pressure steam is superheated. 4 designates a horizontal still having the usual fire box 5, combustion chamber 6 and stack 7. The upper part of the still is equipped with a steam dome 8 having a safety valve 9. Superheated steam is admitted to the still through a pipe, 10, which connects with a delivery pipe 11 lying along the bottom of the still. This delivery pipe is provided with a plurality of curved branch pipes 12 perforated along their lower sides as shown at 13, 13. The pipe 10 is provided with a three way-cock 14 arranged so that the superheated steam may be admitted to the still, or opened to the atmosphere or entirely shut off. The supply pipe 10 is also provided with a check valve 15 in order to prevent any of the residuum backing into the superheater, and causing an explosion. The products of distillation pass from the still into a condenser 16 provided with the usual closed condenser coil 17. The products of distillation are drawn off through a discharge pipe 18 to a suitable receptacle (not shown) where they may be separated and treated as desired. The treatment of the distillates, however, forms no part of the present invention.

Describing now the manner of carrying out such process, the still is charged with semi-asphaltic base petroleum residuum such as is obtained from mid-continent fields. This residuum is preferably of relatively heavy gravity, as for example 12 to 15° Baumé, although residuum of other gravity may be used if desired. After the still is charged it is heated until the residuum attains a temperature of about 450° F., more or less, and superheated steam is then turned in. The steam which has been previously

superheated to a temperature of from about 600° to 700° F. is admitted into the still in large quantities but at relatively low pressure. Ordinarily a pressure slightly in excess of that necessary to overcome the head of the residuum will be sufficient, it being understood however, that the superheated steam shall be introduced into the residuum in such quantities and at such pressure as to blast or thoroughly agitate the latter. By means of the perforated branch pipes the superheated steam is distributed throughout the residuum and intimately mixed with the latter. As the treatment proceeds the temperature of the still may be raised to as high as 700° F. depending upon the character and gravity of the residuum used and upon the grade of product desired. The temperature, however, is at all times kept below that at which the residuum would normally boil or distil. The process is continued until a product of the desired melting point and consistency has been obtained, care always being taken to keep the temperature sufficiently low to avoid any danger of decomposition. This superheated steam passing through and agitating the residuum, in effect, so varies the vapor pressure of the residuum and of the paraffin and vaseline hydrocarbons that the latter are removed from the still at temperatures considerably below that at which they would normally decompose. If the process be carried out far enough the major portion of the paraffin and vaseline hydrocarbons contained in the original residuum can be removed without decomposition or without injuring the asphaltic hydrocarbons remaining. It is well known to asphalt chemists that the presence of these heavy vaseline and paraffin hydrocarbons in asphaltic products is undesirable, as these hydrocarbons are non-cementitious, non-ductile, non-adhesive and greasy in character and in addition impart these undesirable characteristics to the asphaltic hydrocarbons when mixed with the latter. Nevertheless, no artificial asphalts or asphaltic fluxes have heretofore been made from semi-asphaltic base petroleum residuum which were sufficiently free from these deleterious hydrocarbons or their cracked residues to obtain a product of the character in question. It is to be understood that all of the vaseline and paraffin hydrocarbons are not necessarily removed by my process. The softer products naturally will not have as large a percentage of these hydrocarbons removed as will the harder grades, in which the process has been carried on to a further degree, but in either case, a sufficient amount of the paraffin and vaseline hydrocarbons must be removed to obtain a product having the qualities and desired characteristics. I have found however, that in any case it is very advisable, if not necessary to remove from the residuum the greater part of these vaseline, paraffin and analogous hydrocarbons. It will perhaps be better understood and appreciated by a comparison of products produced by this process with those produced by other processes when treating the same residuum. The following analyses of two products made by my process will clearly illustrate the foregoing statement:

|                                        | A.               | B.               |
|----------------------------------------|------------------|------------------|
| Specific gravity at 77° F.....         | Over 1.....      | Over 1.....      |
| Melting point.....                     | 110° F.....      | 130° F.....      |
| Ductility at 77° F.....                | Over 100 cm..... | Over 100 cm..... |
| Penetration at 32° F.....              | 19.....          | 10.....          |
| Penetration at 77° F.....              | 92.....          | 32.....          |
| Penetration at 115° F.....             | Over 450.....    | 213.....         |
| Solubility in carbon disulfid.....     | 99.5.....        | 99.5.....        |
| Solubility in carbon tetrachlorid..... | 99.5.....        | 99.5.....        |

For the penetration tests the well known Dowe standard machine and method was used. For the ductility tests also the well known Dowe briquet molds were used, having a cross section of one square centimeter. The briquets are pulled apart at a standard temperature at the rate of 5 centimeters per minute. These briquets are about 5 centimeters in length. Product A when compared with a commercial air blown asphalt made from the same residuum and having the same penetration or hardness at 77° F. shows many differences. The specific gravity of the product produced by my process is in excess of the specific gravity of the air blown asphalt, while the melting point on the other hand is only about one half as high. The ductility of my product produced by my process is more than fifty times that of the air blown asphalt. While both of these products have the same penetration or consistency at 77° F. as above stated, the penetration of the air blown asphalt at 32° F. is more than three times that of my product. In other words, at 32° F. my product is much harder than is the air blown asphalt product. On the other hand, the penetration of the product produced by my process at 115° F. is about three times that of the product produced by the use of air. In short, at 115° F. air blown asphalt product is still a solid while at the same temperature my product is practically a liquid. Product B when compared with an air blown asphalt having a common basis of comparison varied in a similar manner. Inasmuch as I have compared my product with an air blown asphalt having a common basis of comparison, as for example its consistency at 77° F., such products should have all other characteristics similar, if the products are the same or similar. From the solubility tests above given it is also apparent that there is no material decomposition in my products produced by my new process, and further that no material amount

of carbenes are formed, the presence of carbenes as is well known, indicating the presence of decomposition products. From the foregoing analysis it will also be seen that a 5 product made by this process will contain less than two per cent. of coke.

From the foregoing it will be seen that my process differs radically from the process heretofore known in that in treating 10 residuum of the character in question it produces a product radically different from any heretofore known.

A product produced by my process is particularly adapted for those cases in 15 which an asphaltic product having a high degree of cementitiousness and ductility is required, as for example, in sheet asphalt pavements and the like. Products produced by my process have a ductility at normal 20 temperatures ( $77^{\circ}$  F.) ranging from 25 to over 100 times its cross section, the degree of ductility varying with the consistency of the product. The softer products have a ductility more than 50 times greater than 25 the ductility possessed by any heretofore known asphaltic product of common consistency made from residuum of the same character.

I claim as my invention:

30 1. The process of preparing asphaltic products from semi-asphaltic base petroleum residuum, which consists in heating the residuum in a still at a gradually increasing temperature not in excess of 700 35 degrees F., and simultaneously blasting the charge with a non-oxidizing gas heated to a temperature not in excess of 700 degrees F., so as to distil off a greater part of the paraffin and analogous hydrocarbons contained in the original residuum without material decomposition.

2. The process of preparing asphaltic products which consists in heating semi-asphaltic base petroleum residuum in a still, 45 simultaneously blasting the mass with large quantities of superheated steam, so as to profoundly modify the residuum, removing from such residuum the greater part of the paraffin and analogous hydrocarbons contained therein without material decomposition and without injury to the asphaltic hydrocarbons of the residuum, and thereby producing a product having a marked degree of ductility and cementitiousness.

55 3. The process of preparing asphaltic products which consists in heating semi-asphaltic base petroleum residuum in a still at a temperature not in excess of 700 degrees F., simultaneously, blasting the mass 60 with large quantities of superheated steam, the process being conducted at such temperature as to remove a considerable part of the paraffin hydrocarbons contained in the residuum without material decomposition 65 or injury to the asphaltic hydrocarbons of

the residuum and thereby producing a product having a marked degree of ductility and cementitiousness.

4. The process of preparing asphaltic products which consists in heating petroleum residuum in a still at a temperature not in excess of 700 degrees F., simultaneously blasting the mass with superheated steam at relatively high temperatures but not in excess of 700 degrees F., and at a minimum pressure, removing a considerable part of the paraffin hydrocarbons contained in the residuum so as to produce a product having a high degree of ductility and marked cementitiousness.

5. The process of preparing asphaltic products from asphalt bearing base petroleum residuum, which consists in heating such residuum in a still at a temperature not in excess of 700 degrees F., and simultaneously blasting the mass with large quantities of steam superheated to a temperature not in excess of 700 degrees F. to remove a considerable portion of the paraffin and analogous hydrocarbons, whereby the finished product will contain a substantially greater percentage of unsaturated hydrocarbons than did the untreated residuum and be free of any material decomposition.

6. The process of preparing asphaltic products which consists in charging a still with a mass of asphalt bearing base petroleum residuum, gradually heating said still to a temperature not in excess of 700 degrees F., and during said heating blasting said residuum with large quantities of steam superheated to a temperature not in excess of 700 degrees F., and continuing said treatment until a major portion of the saturated hydrocarbons, *i. e.* those non-removable by concentrated sulfuric acid, have passed out of the still, and without material decomposition.

7. The process of preparing asphaltic products from petroleum residuum, which consists in heating such residuum in a still at a temperature between  $500^{\circ}$  F. and  $700^{\circ}$  F., and simultaneously blasting the mass with large quantities of superheated steam at a temperature not in excess of  $700^{\circ}$  F. 115 and continuing such treatment until a major portion of the saturated hydrocarbons, *i. e.*, those non-removable by concentrated sulfuric acid, has passed out of the still, and in carrying out such process and introducing such quantities of steam and maintaining such temperatures as will avoid any substantial decomposition.

8. The process of distilling asphalt bearing oil by subjecting the same to the action 125 of heat and simultaneously injecting into the mass superheated steam, the degree of heat being sufficiently low and the amount of steam being sufficiently great to produce a solid or semi-solid residue free from the 130

major portion of the paraffin hydrocarbons contained in the untreated residuum and free from any material decomposition.

9. The process of preparing an asphaltic product from an asphalt bearing oil which consists in heating such oil in a still to a temperature above 450 deg. F., blasting the oil with large quantities of superheated steam and continuing the treatment until a large portion of the saturated hydrocarbons *i. e.*, those non-removable by concentrated sulfuric acid, have passed out of the still and regulating the temperature and quantity of superheated steam, so as to avoid the formation of more than two per cent. of coke over and above that which may have been originally contained in the untreated oil.

10. The process of preparing from an asphalt bearing oil an asphaltic product having a relatively high degree of ductility and cementitiousness, which consists in heating said oil in a still to a temperature in excess of 450° F., blasting the heated oil with large quantities of highly superheated steam and continuing the operation until a semi-solid or solid asphaltic product is produced and regulating the temperature and quantities of superheated steam so as to avoid any substantial decomposition in the product.

11. An asphaltic product made from semi-asphaltic base petroleum residuum, said product being free from a greater part of the paraffin and analogous hydrocarbons contained in the residuum and free from any material decomposition, having a relatively great ductility and possessing the characteristics of a product obtained by subjecting the semi-asphaltic base petroleum residuum in a still to the action of heat and superheated steam at temperatures sufficiently low to avoid any material decomposition, *i. e.*, not in excess of 700° Fahrenheit.

12. An asphaltic product made from semi-asphaltic base petroleum residuum, said product being free from a greater part of the saturated hydrocarbons contained in the original residuum and free from any material decomposition, a briquet of such material which is one centimeter square in cross section and 5 centimeters in length having a

ductility ranging from 25 to 100 centimeters at 77 deg. F., the degree of ductility varying with the consistency of the product.

13. An asphaltic flux capable of fluxing indurated natural bitumens such as grahamites and giving to the resultant compound a high degree of ductility and cementitiousness, such flux being formed from semi-asphaltic base petroleum residuum, and having the characteristics of a product obtained by subjecting such residuum to the action of heat and superheated steam at temperatures sufficiently low to remove certain portions of the saturated hydrocarbons without material decompositions, *i. e.*, at temperatures not in excess of 700° Fahrenheit.

14. An asphaltic product made from semi-asphaltic base petroleum residuum, markedly high in its content of unsaturated hydrocarbons, *i. e.*, those removable by concentrated sulfuric acid and markedly lower in its content of saturated hydrocarbons, *i. e.*, those non-removable by concentrated sulfuric acid, than the residuum from which it was derived, free from material decomposition and in general possessing the characteristics of a product obtained by subjecting a semi-asphaltic base petroleum residuum to the action of heat and superheated steam at a temperature below 700 degrees Fahrenheit.

15. An asphaltic product made from petroleum residuum markedly high in its content of unsaturated hydrocarbons, *i. e.*, those removable by concentrated sulfuric acid and markedly lower in its content of saturated hydrocarbons, *i. e.*, those non-removable by concentrated sulfuric acid, than the residuum from which it was derived, free from material decomposition and in general possessing the characteristics of a product obtained by subjecting a petroleum residuum to the action of heat and superheated steam at a temperature below 700 degrees Fahrenheit.

LESTER KIRSCHBRAUN.

Witnesses:

F. L. BELKNAP,  
J. M. LUTZ.